

## UNITED STATES PATENT OFFICE

GEORGE BURKLE HOLDERER, OF SCARSDALE, NEW YORK, AND LE ROY V. CLARK, OF PITTSBURGH, PENNSYLVANIA

## EXPLOSIVE

No Drawing.

Application filed June 8, 1931. Serial No. 543,006.

This invention relates to explosives and more particularly to liquid oxygen explosives.

In the use of liquid oxygen explosives a suitable quantity of carbon or carbonaceous material is placed in a bag and liquid oxygen added thereto, the oxygen being absorbed by the carbon or other carbonaceous material. The cartridges actually used in this manner may be of considerable size and when they are to be used they are placed or dropped in a hole or bore to be exploded, with the detonating material and the charge then tamped. In dropping the cartridge into a hole there is considerable chance of tearing the bag or casing and if this occurs, the loose carbon, which is now used and which is highly charged with oxygen, is released in the form of a dust. As this charge is highly explosive, the risk of premature explosions is very great. In the present invention we propose to form an explosive in which the carbon particles are bound together and dust will, therefore, not be created if the bag or casing is torn in dropping the cartridge into a hole, or in any other way. By binding the carbon particles together we may eliminate the casing, but we prefer to use it to retard evaporation of the absorbed liquid oxygen. We may, however, use a bag or casing of a much lighter material than that heretofore employed and thus reduce the cost of manufacture of the cartridge.

We are aware of prior efforts to produce an explosive consisting of carbonaceous material having absorbed liquid air as an oxidizing medium in which the carbonaceous material is bonded together to form a substantially rigid structure. In the prior art with which we are familiar the carbonaceous material so employed has been in the form of a powder and has been molded in such manner that a non-porous structure would be produced if special precautions were not exercised to give porosity to the material. It has heretofore been proposed to mix the carbonaceous material with an adhesive, sufficient liquid to form a paste and with a ferment, such as yeast or sodium bicarbonate. The pasty mixture so formed is pressed and then baked until a rigid body is obtained, the action and ferment be-

ing relied upon to produce the necessary porosity.

We are also aware of prior efforts to produce liquid oxygen explosives in the form of a rigid body in which a material such as molasses is used and dehydrated or partially dehydrated and mixed with powdered charcoal or carbon-black. We have found that a sufficiently porous, carbonaceous material may be produced in the form of a cake or stick by using carbons or carbonaceous material of a proper character and merely treating it with sufficient binder to hold the particles together without substantially decreasing the porosity of the carbon or carbonaceous material. In our invention we specifically avoid the production of a pasty mass and subsequent molding of this material in such form as would produce a non-porous body if such precautions were not taken to provide for the porosity of the cartridge. In carrying out our invention we employ a carbon in granular form. If powdered carbon is mixed with a binder in liquid form, we have found that the resulting product does not possess sufficient porosity. We, therefore, employ what is commercially known as Bugbird carbon, which we understand is produced in accordance with the Bugbird patents Nos. 1,706,871, 1,779,530 and 1,781,214. As disclosed in these patents the carbonaceous material which we employ preferably consists of granules or particles of such size that the density of the product is equal to about 0.25 to 0.35. The grains of carbon vary considerably in size, the largest being about one-quarter inch in their longest dimension and the size of the granules being such that about 25 per cent of the material will pass through a 100 mesh screen. While the use of Bugbird carbon is proposed, it is to be understood that any other carbon or carbonaceous material in granular form may be employed and the invention is not limited to the use of this particular material. Likewise, the size of the grains may vary over the dimensions set forth above, which are merely by way of illustration.

Our invention resides in the use of a granular, carbonaceous material of the character

set forth above in the production of a solid or molded cartridge having a high degree of absorption for liquid oxygen. In carrying out the invention the carbonaceous material is mixed with a suitable binder. We may employ a starch solution for this purpose and purpose to use a solution containing from 1 to 10 per cent of the starch. In a specific form of the invention a 7 per cent mixture 5 by weight of starch and water was prepared and heated to boiling. The carbon may be sprayed with this solution and then pressed gently in a mold and dried. The resulting cartridge has the ability of absorbing oxygen substantially to the same degree as the carbon in loose form and substantially the same results have been obtained in impact tests to determine the sensitivity of the explosive.

In practicing the invention on a commercial scale, a suitable binder, such as the starch solution set forth above, may be sprayed on the carbon sufficiently to wet it and the carbon in this form filled into the bags or casings in the usual filling machine. The cartridge may then be allowed to dry and the carbon will be sufficiently agglomerated to prevent dusting. When the casing is employed with the cartridge it is not necessary that the cartridge be baked or oven dried to 20 a hard and solid product and better results are obtained if only the usual pressure now applied in filling bags is used so that the carbon particles are merely bonded together sufficiently to prevent dusting if the bag tears 25 when it is dropped into a drill hole. In the commercial use of liquid oxygen explosives substantially 15 per cent of moisture may be retained in the carbon and we therefore propose to avoid drying of the cartridge to complete dryness.

In place of starch any of the usual binders may be employed. The binder must be chosen in consideration of its adhesiveness, its ability to be used in connection with the 45 usual filling machine for liquid oxygen cartridges and its ability to dry or set quickly. It must also be capable of producing a cartridge having sufficient resistance to crushing and it must not adversely affect the ability of the carbon or carbonaceous material to absorb and retain liquid oxygen. Other binders which may be used in place of starch are organic binders, such as gelatin and gluten, various glues and pastes, various 50 sugar or saccharine compounds, resins and gums, such as natural or synthetic resins, gum arabic, phenol and the like, cellulose plastics and lacquers, rubber, waxes and petroleum products, such as tars, pitch and 55 paraffin.

We may also employ inorganic binders, such as sodium silicate, plaster of Paris and the like.

As stated, the essential feature of the invention is the use of carbon or carbonaceous

material in granular form whereby a molded product can be formed by the use of a limited quantity of a binder in which the ability of the carbon or carbonaceous material to absorb and retain liquid oxygen is not seriously impaired. By the use of such a binder and just sufficient pressure to hold the particles together to prevent dusting in case of tearing of the cartridge case or bag in lowering the cartridge into a drill hole, 75 the hazard of carbon dust suspended in an atmosphere of oxygen is eliminated.

We claim:

1. A liquid oxygen explosive material comprising carbonaceous material in granular form and a binder in an amount sufficient to 80 agglomerate the carbonaceous material without appreciably affecting its porosity.

2. A cartridge for liquid oxygen explosives comprising a granular carbonaceous material and a binder in an amount sufficient to 85 agglomerate the carbonaceous material without appreciably affecting its porosity, said cartridge containing approximately 10 per cent of water.

3. A cartridge for liquid oxygen explosives comprising granular carbonaceous material and a starch binder in an amount sufficient to 90 agglomerate the carbonaceous material without appreciably affecting its porosity.

4. A cartridge for liquid oxygen explosives comprising a granular carbonaceous material and an inorganic binder in an amount sufficient to 95 agglomerate the carbonaceous material without appreciably affecting its porosity.

5. A cartridge for liquid oxygen explosives comprising a granular carbonaceous material and an organic binder in an amount sufficient to 100 agglomerate the carbonaceous material without appreciably affecting its porosity.

6. A cartridge for liquid oxygen explosives comprising granular carbonaceous material, the granules being of such size that the longest dimension is approximately  $\frac{1}{4}$  inch and that substantially 25 per cent will pass through a hundred mesh screen, and a binder in an amount sufficient to agglomerate the carbonaceous material without appreciably affecting its porosity, said cartridge containing substantially 10 per cent of moisture.

7. The herein described process which comprises applying a binder in liquid form to granular carbonaceous material in an amount sufficient to agglomerate the carbonaceous material but insufficient to appreciably reduce its porosity, and pressing the material into a cartridge.

8. The herein described process which comprises applying a binder in liquid form to granular carbonaceous material in an amount sufficient to agglomerate the carbonaceous material but insufficient to appreciably reduce its porosity, pressing the material into a car-

tridge and drying the cartridge to a moisture content of substantially 10 per cent.

5 9. The herein described process which comprises applying a starch solution to granular carbonaceous material in an amount sufficient to agglomerate the carbonaceous material but insufficient to materially reduce its porosity and then pressing the carbonaceous material into a cartridge.

10 10. The herein described process which comprises applying an organic binder in a liquid form to carbonaceous material in an amount sufficient to agglomerate the carbonaceous material but insufficient to materially 15 reduce its porosity and then pressing it into a cartridge.

11. The herein described process which comprises applying an inorganic binder in a liquid form to carbonaceous material in an amount sufficient to agglomerate the carbonaceous material but insufficient to materially 20 reduce its porosity and then pressing it into a cartridge.

12. The herein described process which 25 comprises applying a binder in liquid form to granular carbonaceous material in an amount sufficient to agglomerate the carbonaceous material but insufficient to materially 30 reduce its porosity and then filling the material into a cartridge casing to cause agglomeration of the material.

In testimony whereof we affix our signatures.

GEORGE BURKLE HOLDERER.

35 LE ROY V. CLARK.

40

45

50

55

60

65